

## UNITED STATES PATENT OFFICE

2,381,120

METHOD OF REDUCING BARITE IN FLUOR-  
SPAR CONCENTRATE

Walter E. Duncan, Rosiclare, Ill., assignor to  
Mahoning Mining Company, Youngstown, Ohio,  
a corporation of Delaware

No Drawing. Application December 24, 1943,  
Serial No. 515,596

5 Claims. (Cl. 209—167)

My invention in general relates to flotation recovery of fluorspar from fluorspar-bearing ores and is more particularly directed to reduction of the residual amount of barite in the final concentrates when the latter are obtained from ores in which it is present in material quantities.

Many fluorspar-bearing ores contain barite ( $BaSO_4$ ) in amounts running up to 15% or more and when in excess of about 2% it has heretofore been substantially impossible in commercial practice to prevent the appearance of appreciable quantities of it in the final fluorspar concentrates. While the presence of this residual barite is not inimical to use of the concentrates for customary industrial purposes it nevertheless acts as a diluent, and is therefore objectionable through its lowering of the total fluorspar content of a given volume of the concentrate and particularly so when the latter is of "acid-grade," a term generally utilized to designate a concentrate containing over 97% fluorspar ( $CaF_2$ ).

Consequently various methods have been proposed for reducing this residual barite during treatment of ores initially containing over about 2% thereof but as far as I am aware none of them has been highly successful in actual flotation practice, especially when considered from the standpoints of practicability, convenience and operating costs.

I have discovered, however, that by utilization of a suitable reagent it is practicable to first remove by flotation a very large portion of the barite in the ore and to then recover from the tailings of this flotation fluorspar concentrates devoid of barite in objectionable amounts.

A principal object of my invention therefore, is the provision of a novel method of reducing the residual barite in fluorspar concentrates produced from fluorspar ores containing substantial amounts of barite by first removing a large proportion of the latter by flotation in the presence of a suitable reagent and then recovering the fluorspar from the tailings of that flotation.

My invention further comprises the use of a novel reagent for floating the barite during the initial flotation step.

Other objects, purposes and advantages of the invention will hereinafter more fully appear or will be understood from the following description of a preferred manner of its practice.

In performing the invention, which in commercial usage may be most efficiently and satisfactorily carried out as a continuous operation through suitable arrangement of the various flotation cells and other apparatus employed and which may be of any suitable character, the ore

is first ground to a suitable fineness such as —100 mesh and then pulped and floated in water to which has been added a suitable amount of a sodium oleyl sulfate, hereinafter more particularly identified, which acts as an effective collector for the barite, with production of an extremely controllable froth in contradistinction to froths produced by those alkyl sulfates represented by the long chain alcohol sulfates which, though powerful frothers, create froths which are watery, quite stable and not heavily mineralized. In fact, many of the froths produced by use of these other alkyl sulfates are virtually uncontrollable because of their tendency to be voluminous, to become wild and at times to make simply almost barren suds. In contradistinction to these characteristics, however, the froth resulting from employment of the said sodium oleyl sulfate is readily controlled, heavily mineralized with barite and easily manipulated and removed so that the tailings resulting from the flotation contain but little barite and are thus conditioned for the second step incident to the practice of the invention, namely, flotation recovery of their fluorspar content which may be effected by any suitable process, but preferably by that of U. S. Patent 2,168,762, granted August 8, 1939, to Clemmer and Anderson which entails, among other things, the use of quebracho extract as a depressant for the calcite content of the pulp and a fatty acid flotation reagent as a collector for the fluorspar.

As exemplifying the practice of my invention but not by way of restriction or limitation, I shall now refer to results obtained in the treatment of different ores containing, among other things, barite and fluorspar; in each case the ore was first ground to —100 mesh, a batch treatment employed in Examples I and II, and a continuous treatment in Examples III and IV.

## Example I

The ore utilized analyzed with respect to its principal constituent elements as follows:

|          | Per cent |
|----------|----------|
| $CaF_2$  | 61.90    |
| $BaSO_4$ | 14.21    |
| $CaCO_3$ | 20.49    |
| $SiO_2$  | 1.20     |

no sulfides being present. The barite was floated first, using soft water to which for the rougher circuit had been added 1.0 lb. of the sodium oleyl sulfate, 2.0 lbs. sodium silicate, 0.48 lb. citric acid and 1.0 lb. barium chloride per ton of feed; the concentrate was then cleaned three times in a

cleaner circuit with soft water containing 1.3 lbs. sodium silicate per ton of feed. The fluorspar in the tailings of the barite flotation was next floated in accordance with the practice disclosed in said Patent 2,168,762 using soft water to which, for the rougher circuit, had been added 1.0 lb. soda ash, 2.0 lbs. oleic acid and 2.0 lbs. quebracho extract per ton of feed, and the concentrate was then cleaned four times in a cleaner circuit using soft water containing 3.0 lbs. quebracho extract per ton of feed. The following results were obtained:

|                                | Assay, per cent   |                  | Mineral distribution, per cent |                  |
|--------------------------------|-------------------|------------------|--------------------------------|------------------|
|                                | BaSO <sub>4</sub> | CaF <sub>2</sub> | BaSO <sub>4</sub>              | CaF <sub>2</sub> |
| Feed                           | 14.21             | 61.90            |                                |                  |
| Barite final concentrate       | 96.4              | 1.3              | 87.9                           | 0.3              |
| Barite middlings               | 6.1               | 73.0             | 4.6                            | 15.4             |
| Barite rougher concentrate     | 55.9              | 33.3             | 92.5                           | 15.7             |
| Fluorspar final concentrate    | 0.13              | 96.95            | 0.6                            | 72.5             |
| Fluorspar middlings            | 1.34              | 63.39            | 0.6                            | 9.3              |
| Fluorspar rougher concentrates | 0.4               | 92.7             | 1.2                            | 81.8             |
| Tailings                       | 6.1               | 9.5              | 6.3                            | 2.5              |
| Composite                      | 14.2              | 61.2             | 100.0                          | 100.0            |

#### Example II

The ore utilized analyzed with respect to its principal constituent elements as follows:

|                   | Per cent |
|-------------------|----------|
| CaF <sub>2</sub>  | 62.5     |
| BaSO <sub>4</sub> | 13.9     |
| CaCO <sub>3</sub> | 9.7      |
| SiO <sub>2</sub>  | 18.2     |
| Zn                | 1.1      |
| Pb                | 0.5      |

Again the barite was floated first, using soft water to which for the rougher circuit had been added 1.0 lb. sodium oleyl sulfate, 2.0 lbs. sodium silicate, 1.0 lb. barium chloride and 0.5 lb. citric acid per ton of feed; the concentrate was then cleaned three times in a cleaner circuit with soft water containing 1.6 lbs. sodium silicate per ton of feed. The fluorspar in the tailings of the barite flotation was next floated as in Example I using soft water to which, for the rougher circuit, had been added 1.6 lbs. soda ash, 1.0 lb. oleic acid and 0.8 lb. quebracho extract per ton of feed and the concentrate was then cleaned three times in a cleaner circuit using soft water containing 0.8 lb. quebracho extract per ton of feed. The following results were obtained:

|                                | Assay, per cent   |                  | Mineral distribution, per cent |                  |
|--------------------------------|-------------------|------------------|--------------------------------|------------------|
|                                | BaSO <sub>4</sub> | CaF <sub>2</sub> | BaSO <sub>4</sub>              | CaF <sub>2</sub> |
| Feed                           | 13.90             | 62.5             |                                |                  |
| Barite final concentrates      | 92.14             | 3.77             | 59.9                           | 0.5              |
| Barite middlings               | 11.50             | 52.30            | 15.8                           | 16.3             |
| Barite rougher concentrates    | 35.9              | 37.4             | 72.7                           | 16.8             |
| Fluorspar final concentrates   | 0.20              | 97.09            | 0.7                            | 62.9             |
| Fluorspar middlings            | 1.28              | 59.24            | 1.4                            | 17.9             |
| Fluorspar rougher concentrates | 0.5               | 85.0             | 2.1                            | 80.8             |
| Tailings                       | 26.78             | 11.68            | 25.2                           | 2.4              |
| Composite                      | 13.90             | 62.50            | 100.00                         | 100.00           |

#### Example III

The ore utilized analyzed with respect to its principal constituent elements as follows:

|                   | Per cent |
|-------------------|----------|
| CaF <sub>2</sub>  | 61.1     |
| BaSO <sub>4</sub> | 17.9     |
| CaCO <sub>3</sub> | 16.7     |
| SiO <sub>2</sub>  | 1.1      |

A continuous instead of batch treatment was employed, the barite being floated first using soft water to which, for the rougher circuit, had been added 2 lbs. sodium silicate and 0.5 lb. sodium oleyl sulfate per ton of feed and the concentrates obtained were cleaned in a cleaner circuit using soft water containing 1.2 lbs. sodium silicate per ton of feed. The tailings following this treatment were then floated for fluorspar in accordance with the practice disclosed in said Patent 2,168,726, using soft water to which, for the rougher circuit, had been added 0.32 lb. oleic acid, 0.6 lb. of sodium carbonate and 1.5 lbs. quebracho extract per ton of feed. The concentrates were then cleaned in a cleaner circuit using soft water containing 1.8 lbs. quebracho extract per ton of feed. The following results were obtained:

|                              | Assay, per cent   |                  | Mineral distribution, per cent |                  |
|------------------------------|-------------------|------------------|--------------------------------|------------------|
|                              | BaSO <sub>4</sub> | CaF <sub>2</sub> | BaSO <sub>4</sub>              | CaF <sub>2</sub> |
| Feed                         | 17.9              | 61.1             |                                |                  |
| Barite final concentrates    | 71.3              | 18.4             | 92.4                           | 7.0              |
| Barite tailings              | 1.8               | 74.0             | 7.6                            | 93.0             |
| Fluorspar final concentrates | 0.8               | 92.9             | 2.5                            | 88.4             |
| Fluorspar final tailings     | 4.9               | 14.9             | 5.1                            | 4.6              |

#### Example IV

The ore utilized analyzed with respect to its principal constituent elements as follows:

|                   | Per cent |
|-------------------|----------|
| CaF <sub>2</sub>  | 63.88    |
| BaSO <sub>4</sub> | 9.30     |
| CaCO <sub>3</sub> | 7.50     |
| SiO <sub>2</sub>  | 11.68    |
| Zn                | 0.66     |
| Pb                | 0.05     |

As in Example III the barite was floated first using soft water to which for the rougher circuit had been added 0.5 lb. sodium oleyl sulfate, 1.3 lbs. sodium silicate, 1.0 lb. soda ash and 0.5 lb. citric acid per ton of feed and the concentrate was cleaned in a cleaner circuit using soft water containing 0.07 lb. sodium silicate. The tailings following this treatment were then floated for fluorspar as in that example, using soft water to which, for the rougher circuit, had been added 1.15 lbs. oleic acid and 0.9 lb. quebracho extract per ton of feed, and were then cleaned in a cleaner circuit using soft water containing 0.30 lb. quebracho extract per ton of feed. The following results were obtained:

|                              | Assay, per cent   |                  | Mineral distribution, per cent |                  |
|------------------------------|-------------------|------------------|--------------------------------|------------------|
|                              | BaSO <sub>4</sub> | CaF <sub>2</sub> | BaSO <sub>4</sub>              | CaF <sub>2</sub> |
| Feed                         | 9.30              | 63.88            |                                |                  |
| Barite final concentrates    | 91.84             | 1.75             | 88.3                           | 0.3              |
| Barite tailings              | 1.19              | 67.00            | 11.7                           | 99.7             |
| Fluorspar final concentrates | 0.50              | 96.34            | 2.8                            | 83.0             |
| Fluorspar final tailings     | 2.16              | 26.78            | 8.9                            | 16.7             |

The sharpness of separation effected by the flotation in the presence of the sodium oleyl sulfate is readily apparent from these examples for with a barite content of 14.21% and a fluorspar content of 61.90% in the feed, the barite final concentrate showed only 1.3% CaF<sub>2</sub> against 96.4% BaSO<sub>4</sub> in Example I; with a barite content of 13.9% and a fluorspar content of 62.5% in the feed, the barite final concentrate showed only 3.77% CaF<sub>2</sub> against 92.14% BaSO<sub>4</sub> in Example II,

while in Example III with 17.9% barite and 61.1% fluorspar initially present, the barite final concentrate showed 18.4%  $\text{CaF}_2$  against 71.3%  $\text{BaSO}_4$ , and in Example IV, 1.75%  $\text{CaF}_2$  and 91.84%  $\text{BaSO}_4$  against 9.30% barite and 63.88% fluorspar in the feed.

It will be noted that in Examples I and II small amounts of citric acid and barium chloride were used in the flotation of the barite and in Example III a small amount of citric acid, but these reagents are not essential for satisfactory results although sometimes desirable to eliminate the necessity for protracted cleaning; thus the advantages obtainable by the use of the invention are in no way dependent on the presence or absence of these reagents in the barite flotation since results comparable to those given in these examples may be obtained in their absence by merely increasing the number of cleanings prior to the flotation for fluorspar.

As far as I have been able to determine by extended research, optimum results in reduction of residual barite in the final fluorspar concentrate are obtainable only by employment of sodium oleyl sulfate responding to the formula



which may be partially written structurally as



and which is exemplified by materials now marketed by E. I. du Pont de Nemours & Company and by Onyx Oil and Chemicals Company respectively under the trade names or brands "Duponol LS" and "Aurinol," this particular sodium oleyl sulfate when used as a collector apparently tending to form difficultly soluble compounds with the barite but not with the calcium minerals such as fluorspar and calcite ( $\text{CaCO}_3$ ) present in the ore; the advantageous characteristics of the froth engendered by its use have already been mentioned.

As hitherto pointed out, when the barite content of the feed ore is not materially in excess of about 2% recovery of a final fluorspar concentrate with but a comparatively small amount of residual barite can be obtained by flotation of the suitably ground ore in accordance with the disclosure of said Patent 2,168,762, probably because with this high ratio (from about 30:1 and up) of fluorspar to barite the latter is starved or crowded out during the flotation for fluorspar and forced into the tailings. But when the barite is in excess of the amount mentioned this effect is not sufficient to enable the production of a final fluorspar concentrate containing but little residual barite. It therefore seems reasonable to assume that a somewhat similar result takes place when in accordance with the present invention sufficient of the barite is removed by the initial flotation to establish a barite-fluorspar ratio in the tailings of the order just mentioned, thus enabling a material part of the remaining barite to be starved or crowded out during the ensuing flotation for fluorspar with consequent reduction to a minimum of the residual barite in the final concentrate. It follows that the present invention is of maximum utility when the barite content of the ore exceeds about 2% as by its employment a final fluorspar concentrate of acid or substantially acid-grade can readily be produced from ore of that character.

In the aforesaid examples soft water was em-

ployed and is ordinarily to be preferred; hence if only hard water is available it is desirable to soften it by means of a lime-soda or a zeolite treatment, although successful practice of the invention is not dependent upon the use of water of zero or substantially zero hardness. I also prefer to maintain the pH in the flotation circuit between 8.0 and 8.6 but it is to be understood this range is stated merely as indicative of the best way I have found of practising the invention and not as constituting a limitation upon it.

Moreover, while I have herein described my invention with considerable particularity and have given certain examples of its practice, it will be understood that I have done so only for purposes of illustration and not with a view to limiting or restricting it in any manner, as other ways of performing it in accordance with differing operating conditions or with ores of various characters will readily occur to those skilled in the art and may be utilized if desired without departing from the spirit and scope of the invention as defined in the appended claims.

Having thus described my invention, I claim and desire to protect by Letters Patent of the United States:

1. The method of reducing residual barite in fluorspar concentrates derived from ores containing barite in excess of about 2%, which comprises pulping the ground ore with water, floating the pulp in the presence of sodium oleyl sulfate of the formula



35 collecting the barite concentrates resulting from said flotation and subjecting the flotation tailings to agitation in the presence of a soap forming higher fatty acid and quebracho extract to thereby concentrate the fluorspar and induce a further separation therefrom of residual barite in said tailings.

2. In the recovery of fluorspar concentrates by flotation from fluorspar-bearing ores containing barite in excess of about 2%, the steps of pulping the ground ore with water containing sodium oleyl sulfate of the formula



and agitating the mixture to produce a barite-bearing froth, removing said froth and then agitating the tailings of said flotation in the presence of a fatty acid of more than twelve carbon atoms and quebracho extract to thereby form a fluorspar-containing froth and induce further separation between the barite and fluorspar in said tailings.

3. In the recovery of fluorspar concentrates by flotation from fluorspar-bearing ores containing barite in excess of about 2%, the steps of pulping the ground ore with water containing sodium oleyl sulfate of the formula



and agitating the mixture to produce a barite-bearing froth, removing said froth and then agitating the tailings of said flotation in the presence of a fatty acid of more than twelve carbon atoms and quebracho extract to thereby form a fluorspar-containing froth and induce further separation between the barite and fluorspar in said tailings, removing the froth and recovering the fluorspar concentrate therefrom.

4. In the production of fluorspar concentrates from fluorspar-calcite-bearing ores containing barite in an amount exceeding about 2%, the

steps of first pulping the ground ore with water containing sodium oleyl sulfate of the formula



agitating the mixture to produce a barite-bearing froth, removing said froth, and then recovering fluorspar concentrates from the tailings of said flotation by flotation concentration in the presence of a soap forming higher fatty acid and a tannin containing calcite depressing reagent.

5. That method of reducing the residual barite in fluorspar flotation concentrates derived from fluorspar-bearing ores containing barite in ex-

cess of about 2%, which comprises first pulping the ground ore with water containing per ton of feed about 2 lbs. of



as a collector for the barite, agitating the mixture to produce a barite-containing forth, removing the froth, and then subjecting the tailings of the flotation to flotation concentration in the presence of oleic acid and quebracho extract to recover concentrates therefrom containing  $\text{CaF}_2$  and residual barite not exceeding about 2%.

WALTER E. DUNCAN.